

July 6, 1965

A. R. RONZIO ET AL  
PREPARATION OF PARAFFIN WAX FOR UTILIZING  
ITS THERMAL EXPANSION PROPERTIES

3,193,600

Filed Nov. 25, 1960

3 Sheets-Sheet 1



FIG. 1.



FIG. 2.



FIG. 3.



FIG. 3a.

INVENTORS.

ANTHONY R. RONZIO  
JOHN F. SHERWOOD

BY *Bertha L. McGregor*  
ATTORNEY

July 6, 1965

A. R. RONZIO ET AL  
PREPARATION OF PARAFFIN WAX FOR UTILIZING  
ITS THERMAL EXPANSION PROPERTIES

3,193,600

Filed Nov. 25, 1960

3 Sheets-Sheet 2



FIG. 4.



FIG. 5.



FIG. 6.



FIG. 7.

INVENTORS.

ANTHONY R. RONZIO  
JOHN F. SHERWOOD

BY *Bertha L. MacGregor*  
ATTORNEY

July 6, 1965

A. R. RONZIO ET AL

3,193,600

PREPARATION OF PARAFFIN WAX FOR UTILIZING  
ITS THERMAL EXPANSION PROPERTIES

Filed Nov. 25, 1960

3 Sheets-Sheet 3



FIG. 8.



FIG. 9.32



FIG. 10.



FIG. 11.

INVENTORS.

ANTHONY R. RONZIO  
JOHN F. SHERWOOD

BY Bertha L. McGregor  
ATTORNEY

1

3,193,600

**PREPARATION OF PARAFFIN WAX FOR UTILIZING ITS THERMAL EXPANSION PROPERTIES**  
Anthony R. Ronzio, Littleton, and John F. Sherwood, Golden, Colo.; said Ronzio assignor to Thermal Hydraulics, Inc., Denver, Colo., a corporation of Colorado  
Filed Nov. 25, 1960, Ser. No. 71,564  
7 Claims. (Cl. 264—102)

This invention relates to preparation of paraffin wax for utilizing its thermal expansion properties. More particularly, the invention relates to the pre-treatment of paraffin wax for the purpose of improving its capacity to impart motion to mechanisms by expansion of the wax. The expansion properties of wax may also be utilized for the forming of metal products.

Paraffin wax, pre-treated as hereinafter described, may be encased in a high pressure cylinder and heated to actuate reciprocating means in the cylinder for operating dampers, valves, shutters, pumps and other devices.

The thermal expansion of commercial paraffin wax has been utilized heretofore for imparting motion to mechanisms, such, for example, as shown in U.S. Patent No. 2,815,642, December 10, 1957, to John F. Sherwood. In efforts to increase the efficiency of commercial paraffin waxes for actuating mechanisms and for other purposes, such, for example, as the forming of metal products, we have discovered that the composition of waxes can be altered and the thermal expansion properties of the waxes thereby substantially improved.

By experiments which will be described hereinafter, we have determined that paraffin wax contains dissolved hydro-carbon gases and that molten paraffin wax absorbs oxygen from the air. Further, we have ascertained that the presence of these gases in the paraffin wax heretofore used to actuate mechanism lessens the expansion and pressure producing capacities of the wax when heated, and results in a gas cushion which resists the return movement of the pressure actuated means.

Therefore an important object of the invention is to devise methods of preparing paraffin wax for utilizing its expansion properties by pre-treatment which frees contained gases and oxygen from the wax and prevents absorption of oxygen from the air by the degassed wax. When the wax, pre-treated as described herein, is sealed in a high pressure cylinder or mold and subjected to heat, it exhibits high expansion and pressure exerting capacities compared to commercial paraffin waxes. When cooled, the wax produced by our invention contracts without formation of gases. When sealed in a cylinder, the contraction of our pre-treated wax results in a vacuum zone located axially of the cylinder which facilitates the return stroke of pressure actuated means in the cylinder.

The valves, dampers, shutters and other mechanisms referred to herein, which may be operatively connected to pistons or plungers actuated by the thermal expansion of wax encased in a high pressure cylinder, usually are designed to function automatically in response to thermostatic controls at different temperatures, sometimes within narrow ranges of temperatures. Therefore the production of wax having the desired melting point or range, as well as optimum expansion and contraction properties, is another important object of our invention.

Paraffin wax is a mixture of hydrocarbon compounds belonging to three distinct systems: the straight or long chain waxes, branched chain waxes and naphthenic waxes. The long chain paraffins have higher melting points than the branched chain, and the naphthenic paraffins have the lowest melting points for components having the same

2

number of carbon atoms. The separation of hydrocarbons for the purposes of this invention may be based on boiling point or on structure, i.e. the clathrate forming compounds which in general, are long chain hydrocarbons.

The paraffin wax known commercially as Eskar-R40, for example, is suitable for treatment by our process, and therefore the experiments described herein were performed with respect to this wax.

10 The aforementioned and other objects and advantages of the invention will become apparent from the drawings and following specification.

In the drawings:

FIG. 1 shows diagrammatically a vacuum distillation apparatus used in Experiment 1.

FIGS. 2 and 3 show diagrammatically the apparatus employed in Experiment 2.

FIG. 3-a is a graph showing volume increase of a wax sample at different temperatures.

20 FIGS. 4, 5, 6 and 7 show diagrammatically the apparatus employed in Experiments 4, 5, 6 and 7, respectively.

FIG. 8 shows diagrammatically the steps of the method used to mold paraffin wax, pre-treated according to this invention, and to encase the molded wax in a high pressure cylinder for actuating a piston embedded in the wax.

FIG. 9 is a plan view of the mold included in FIG. 8.

FIG. 10 is a vertical sectional view in the plane of the line 10—10 of FIG. 9, on an enlarged scale.

30 FIG. 11 is a vertical sectional view showing the method of encasing the molded wax and parts embedded therein in a high pressure cylinder.

*Experiment 1.*—In order to study the behavior of narrow cut fractions of a selected paraffin wax, a vacuum fractional distillation of Eskar-R40 was made by the following procedure: A 200 g. sample was fractionally distilled through a vacuum distillation apparatus shown in FIG. 1. The still pot was heated with an oil bath to obtain uniform and even heat. The oil bath temperature gradually rose during the course of this distillation from 230° C. to 265° C. As the heating progressed there was a vigorous evolution of gas. The Vigreux column was warmed with turns of Nichrome wire which in turn was controlled with a Variac transformer.

40 The vacuum in the distillation apparatus was broken two times in order to change distillate receivers. The distillation temperatures changed in both instances even though the pot was allowed to cool to about 100° C. before admitting air.

45 The fractions collected in Experiment 1 are shown in the following Table 1:

Table 1

| 55 | Fraction No. | Range, °C. | Weight, grams | MP Range | Remarks                            |
|----|--------------|------------|---------------|----------|------------------------------------|
| 60 | 1            | 130-175    | 13.61         | 53-56    | Vacuum broken to change receivers. |
|    | 2            | 175-180    | 20.21         | 54-55.5  |                                    |
|    | 3            | 180-185    | 14.64         | 55.5-56  |                                    |
|    | 4            | 185-190    | 22.92         | 55.5-57  |                                    |
|    | 5            | 190-195    | 21.30         | 57.5-64  |                                    |
| 65 | 6            | 185-190    | 14.64         | 58.5-61  | Do.                                |
|    | 7            | 190-200    | 32.36         | 59-63    |                                    |
|    | 8            | 200-210    | 28.92         | 61-65    |                                    |
|    | 9            | 200-210    | 11.39         | 59-66    |                                    |
|    | 10           | Residue    |               |          |                                    |

*Experiment 2.*—The rate of expansion of the Eskar-R40 wax in response to temperature changes was deter-

mined by the following described experiment. The apparatus shown in FIGS. 2 and 3 was fabricated of Pyrex glass. The dialotometer, FIG. 2, was calibrated with water. The dried reservoir 10 was filled with wax to the mark indicated by the arrow.

The tube was then attached to the vacuum system and the wax melted and cooled until completely degassed and no empty space was present. Water was added to the reservoir to the fiducial mark and the assembly then attached to the apparatus as shown in FIGURE 3.

A series of determinations were made using the boiling point of solvents to maintain a constant temperature. Progress in the work showed it was necessary to determine points on the curve at closer intervals. Mixtures of methylene chloride, B.P. 40.1°, and ethylene chloride, B.P. 83.5°, were therefore used. The data obtained is shown in the following table.

Table 2

| No. | B.P., degrees | Time  | Volume Increase ml. | Percent-age Change | Remarks                  |
|-----|---------------|-------|---------------------|--------------------|--------------------------|
| 1   | 22            | 8.30  |                     |                    | Room temperature.        |
| 2   | 36            | 9.30  | .460                | 1.6                |                          |
| 3   | 40.5          | 9.50  | .280                | 2.5                |                          |
| 4   | 45.0          | 10.10 | .310                | 3.6                |                          |
| 5   | 51            | 10.30 | .235                | 4.4                |                          |
| 6   | 54.5          | 11.20 | .175                | 5.0                |                          |
| 7   | 55.6          | 11.40 | .125                | 5.6                |                          |
| 8   | 58            | 12.30 | .795                |                    | Began to melt discarded. |

The data compiled in Table 2 together with data obtained by observing the volume of liquid paraffin at the boiling points of acetone, alcohol, water and toluene, was used to plot the graph shown in FIG. 3-a. As indicated by the graph, the results of this experiment showed that a break occurs in the curve at 45° C., indicating a change of phase, but the change is minor. The significant change in volume occurs at the melting point of the wax which occurred within the range between 54-60° C. This 11% change in volume is pronounced and indicates that as the purity of the wax is increased, the range of melting can be reduced materially so that the change in volume will occur rather sharply.

*Experiment 3.*—In order to determine the amount of contraction upon cooling in the various fractions of the wax, an experiment was conducted with respect to Fractions 1, 5 and 9 of Table 1. Samples of the three fractions were placed in graduated tubes and weighed. The tubes were then connected to the vacuum system and were melted by immersing in boiling water. After 30 minutes the volume was read while still heated to 95.5°.

Upon cooling, the wax samples solidified and contracted leaving a cavity in the center of the tube. This cavity was usually filled with a solidified foam of wax, indicating dissolved gases separated from solution when the wax solidified. The wax was again attached to the vacuum line and melted, then cooled. This was repeated until gas was no longer given off upon cooling. As many as four cycles were necessary to attain this characteristic.

The tubes were then removed from the vacuum line and distilled water was added from a buret to give a quantitative value to the amount of contraction. Sufficient water was added to bring the reading equal to the volume the wax occupied at the temperature of boiling water.

The contraction measured was that observed in going from 95.5° C. (the boiling point of water) to room temperature 22° C.

Fraction 1:

B.P. 130-175° C.; wt. 13.61 g. (6.80% of sample)  
Contraction found: 6.8%

Fraction 5:

B.P. 190-195° C.; wt. 21.30 g. (10.65%)  
Contraction found: 12.45%

## Fraction 9:

B.P. 200-210° C.; wt. 11.39 g. (5.69%)  
Contraction found: 13.66%

5 It was noted in this experiment that gas was given off when the liquid wax solidified. This became apparent as a solid foam of small bubbles in the center of the wax. Upon remelting the wax while under vacuum, these bubbles rose to the surface and were removed by a pump. It was observed that some of the bubbles decreased in size while rising in the liquid, indicating that some gas redissolved. Therefore it was necessary to either repeat the melting-freezing process on the wax while under vacuum, or heat the wax to 150° C. The latter method caused considerable wax loss due to violent evolution of gas.

20 The data obtained from the experiments described with respect to melting points and expansion and contraction rates in response to temperature changes, enable the user to select the paraffin fraction suitable for embodiment in a given thermally controlled mechanism or for other purposes.

25 The next step of our process is the result of experiments which indicate that paraffin wax contains hydrocarbon gas and that molten paraffin wax absorbs oxygen from the air. The presence of these gases in wax deleteriously affects their expansion and contraction properties, and if employed to impart movement to mechanisms, the gases lessen the thermal expansion efficiency 30 of the wax for exerting pressure to actuate said mechanisms and resist the return stroke of the mechanisms when heat is withdrawn and the wax contracts.

35 The following described experiments indicate that hydrocarbon gas is present in wax and is released at about 140° C., or under high vacuum at a temperature of 95° C.; that molten paraffin wax absorbs oxygen from the air and that the oxygen is released slowly when the wax is melted. Unless the wax employed for thermal expansion is freed of gases before being encased, the gases will be released within the pressure cylinder when the contained wax is subjected to heat in the normal operation of the mechanisms.

40 *Experiment 4.*—This experiment was made to determine the kind of gas present in paraffin wax. A quantity of shavings of Eskar-R140, 131.2 g. was placed in a flask and attached to a vacuum system, a diagram of which is shown in FIGURE 4. The vacuum system used is capable of giving very high vacua and includes both a mechanical and diffusion pump 11.

45 After a good vacuum was established in the system, the flask 12 containing the wax was heated in a water bath while trap 13 of the system was cooled with liquid nitrogen. The vacuum was applied as long as gas was evolved by the wax. The system was then opened and flask 12 was allowed to cool in air, and weighed when at room temperature. The loss in weight was less than 0.1 g. which would correspond to less than 0.08% dissolved gas.

50 The material frozen out with liquid nitrogen was a mixture of condensed gases. As the tube, removed from the trap 13, was allowed to warm the majority of the material in the form of a white film was sublimed off and a sweetish odor of hydrocarbon was present. A very small portion, when observed with a magnifying glass, was in the form of minute droplets. These also quickly 55 evaporated off. The odor of hydrocarbon gas was still present. A few milliliters of water was added and the cylinder was shaken. A strip of universal pH paper was added to the solution. There was no change in color, indicating that any volatile acid, if present, was insufficient to change the pH of the solution.

60 This experiment indicated (a) that a hydrocarbon gas, identified by a smell, is present in the wax and is removed under high vacuum at a temperature of 95° C.; (b) a fraction of the hydrocarbon material isolated becomes liquid

before evaporating off; and (c) any acid, if present, is insufficient to change the color of Hydron pH paper.

*Experiment 5.*—An additional experiment was made to further evaluate the observations made in Experiment 4.

(a) When 29.9965 g. of wax was placed in a tared flask, which was attached to the vacuum system and heated with a water bath (95° C.), completely degassed, cooled and weighed again, while still under vacuum, a loss in weight was observed which amounted to 0.0060 g. (0.02%).

(b) The wax was remelted and allowed to solidify in the open air. The flask containing the wax was then attached to the vacuum system shown in FIGURE 5. After evacuation was complete, the pumps were closed off from the vacuum system and the flask containing the wax was heated with a water bath. Gas was given off. When evolution of gas ceased, the wax was allowed to cool to room temperature and the system was allowed to stand overnight. The system, after equilibrium was established showed a pressure of 10 mm. of gas pressure.

Experiment 5(a) indicates that the dissolved hydrocarbon gas amounts to 0.02%.

Experiment 5(b) indicates that molten wax will absorb a gas from air which is then given off at 95° C.

*Experiment 6.*—To establish the nature of gases which are dissolved in paraffin, apparatus shown in FIG. 6 was fabricated and assembled.

A gentle stream of air was pulled through the apparatus with suction. This air was purified (CO<sub>2</sub> removed) by tube 14 filled with Ascarite (a CO<sub>2</sub> absorbent). The gas was then led to the bottom of flask 15 which contained 200 g. of paraffin in the form of lumps. Flask 15 was immersed in a basin of cold water which could be heated with an electric heater when desired. The gas was then led through tube 16 filled with glass wool. This serves to retain any spray or fine particles of wax entrained in the gas stream. Then the gas was passed through tube 17 which was also filled with Ascarite. This tube will absorb any carbon dioxide gas given off by the wax. The gas stream was then passed through a quartz tube 18 which contained a filling of copper oxide which was heated to red heat with burner 19.

At red heat copper oxide, CuO, reacts with hydrocarbon gases to give carbon dioxide and water. Using ethane as an example of the gas we would then have the equation: CH<sub>3</sub>—CH<sub>3</sub>+7CuO→7Cu+2CO<sub>2</sub>+3H<sub>2</sub>O. The oxygen in the air would then combine with the hot copper to regenerate copper oxide.

The gas was then passed through a saturated solution of barium hydroxide contained in flask 20. This reagent will react with carbon dioxide to give insoluble barium carbonate according to the following equation:



Tube 21 is a guard tube filled with Ascarite and serves to remove the CO<sub>2</sub> from the air should the gas stream be blocked in some manner and a vacuum appear in the system causing outside air to be drawn into flask 20.

All rubber stoppers and rubber tubing were boiled in 10% caustic, washed with distilled water and dried at 100° C. before use to remove any organic and inorganic volatile material which might nullify the results.

The assembly was purged by drawing air through the equipment at the same rate to be used later in the experiment. After 30 minutes only a very slight cloudiness appeared in flask 20.

The contents of flask 20 were then replaced with fresh barium hydroxide solution while the flask 15 was warmed with boiling water to melt the wax. Air was pulled through the melted wax for 1 hour at a rate of 3 bubbles/sec. No cloudiness appeared in flask 20 indicating no hydrocarbon was being evolved.

The water bath surrounding flask 15 was removed and the flask was heated directly with the electric heater.

At about 140° C. cloudiness began to appear in flask 20, indicating a hydrocarbon was being freed by the paraffin. This evolution of gas was more rapid above this temperature. Heating was terminated after 30 minutes of heating.

This experiment indicated that paraffin contains a dissolved hydrocarbon which is not given off at the boiling point of water (95.5° C.), 40 degrees above the melting point of the wax, but is freed at 140° C., and that this hydrocarbon is, however, released at 95° C. under high vacuum.

*Experiment 7.*—Since wax degassed under vacuum was shown to absorb a gas from air when allowed to cool in air, it was desirable to know whether oxygen or nitrogen (the two constituents of air) was being dissolved.

The apparatus shown in FIGURE 7 was then assembled and used in this experiment. Nitrogen from a compressed gas cylinder attached to a regulator was led into wash bottle 22. Fine regulation of the gas stream was made with screw clamp 23. Wash bottle 22 contained about 200 ml. of a strong potassium pyrogallate solution (PPG). This solution reacts with oxygen and serves at this point to absorb all trace of oxygen in the stream of nitrogen. The gas stream then is led to the bottom of flask 24 which contained 200 g. of paraffin in the form of lumps. The stream of nitrogen was then led into wash bottle 25 which also contained pyrogallate. Wash bottle 26 contained water only and served as a guard bottle to keep air from bottle 25.

The apparatus was purged for 30 minutes with a flow of nitrogen gas. A trace of oxygen was removed from the nitrogen indicated by a slight darkening of color. The solution in 25 was replaced with fresh solution. After 30 minutes solution in 25 was almost black indicating much oxygen was present.

The wax was then melted by heating the water around the flask 24 with the heater. A fast stream of nitrogen was then used to purge the system (20 minutes). The pyrogallate in 25 was replaced with fresh solution and the experiment was continued. The solution turned black in 10 minutes.

This experiment indicate that wax degassed under vacuum absorbs oxygen from air when allowed to cool in air, and that the oxygen is released slowly when the wax is melted.

Therefore, after selection of a suitable wax, the next step of our process is to free the wax of dissolved hydrocarbon gas and oxygen by pre-heating the wax, and, following the degassing procedure, to prevent absorption by the wax of oxygen from the air by maintaining the degassed wax under vacuum. The temperature at which the wax is degassed before being encased in a sealed cylinder depends on the conditions under which the thermally controlled unit is intended to operate, as more fully explained hereinafter. Before encasing the pre-treated wax in a sealed cylinder, we maintain the degassed wax in molten state under vacuum before and during a molding operation. Preferably we embed a piston together with an electrical filament holder and filament wound thereon in the molten degassed wax under vacuum. This is done by first placing the piston and filament holder with filament wound thereon in a mold and pouring the molten pre-treated wax into the mold under vacuum to cover and embed the said parts and to completely fill the mold cavity. The piston and filament holder with filament thereon may be of the construction shown in the co-pending application of John F. Sherwood, Serial No. 51,110, for Thermally Controlled Expansible Means for Imparting Motion to Mechanism.

FIG. 8 shows diagrammatically a reservoir 30 containing degassed molten wax under vacuum, pre-treated in accordance with this invention, a valved conduit 31 for conveying the wax under vacuum to a two part mold 32 and vacuum producing means. The mold 32, as shown in FIGS. 9 and 10, is provided with four cavities 33 com-

municating with a wax distribution chamber 34 into which wax is fed by the conduit 31. Any desired number of cavities 33 may be provided.

An electrical filament holder 35 with filament 36 wound thereon is placed in each cavity 33. An electrical conductor 37 extends from the filament 36 into the connector 38 which protrudes beyond the bottom of the lower mold part 39. The upper mold part 40 is provided with sealed openings through which extend pistons 41 to be embedded in the wax in each cavity 33. For clarity, one piston 41 is shown in lowered, embedded position while another is shown in raised position in FIG. 10, but it will be understood that the molten pre-treated wax is forced into the cavities 33 from the distribution chamber 34 by the pressure piston 42 therein to completely fill the cavities 33 while the pistons 41 are in raised positions. When the wax has cooled, the pistons 41 are forced downwardly into the wax filled cavities whereby the wax is compressed. All the foregoing steps are performed while the wax is maintained under vacuum. When the wax has solidified in each cavity 33 there has been formed a cylindrical wax unit which includes the embedded filament holder 35 with filament 36 wound thereon, the conductor 37 and connector 38, and also the piston 41 partially protruding from one end of the unit. The adjustable bleeder valves 43 permit passage of air out of the mold cavities as they become filled with wax under vacuum.

The cylindrical wax units indicated as a whole at 44 are removed from the mold 32, ready for insertion in high pressure cylinders such as the one indicated at 45, supported in die 46 of FIG. 11, which is drawn on a slightly larger scale than FIG. 10. The insertion of each unit 44 into a cylinder 45 is performed with the aid of vacuum 47 to draw the unit 44 by suction into the cylinder 45 and establish vacuum in the cylinder. The wax unit 44 then includes the parts embedded therein, together with the conductor 37, connector 38, and the opposite end plate 48. When the unit 44 is in place, the reduced diameter portion 49 of the wax and the protruding end of the piston 41 fit in the cylinder portion 50 and bear against the rubber pad 51 in the bottom of the die 46. The end plate 48 fits in the cylinder 45 and when sealed thereon, closes the cylinder at that end.

Reverting now to the pre-treatment of the selected wax for the purpose of degassing the wax before encasement in a high pressure cylinder, such for example as the cylinder 45 shown in FIG. 11, and preventing formation of gases under normal operating conditions to which the thermally controlled unit may be subjected, we have noted that dissolved gases are freed from the wax by pre-heating to approximately 140° C., or, under high vacuum to approximately 95° C., and that if the unit is required to operate under conditions where the temperature in the high pressure cylinder 45 does not exceed 95° C., the wax functions efficiently by expansion to impart required motion to the piston 41, and contracts when cooled without giving off gases.

However, when the thermal units are required to operate under temperature and load conditions which create much higher temperatures in the high pressure cylinders 45, it is necessary to pre-heat the wax to temperatures above the predetermined operating temperatures of the units to free dissolved gases which otherwise would be given off at said operating temperatures in the cylinders, and then to maintain the degassed wax under vacuum until it has been molded and solidified for insertion in the cylinders 45.

It is known in the art of isolating wax from petroleum, that chlorinated hydrocarbons are employed in the purification processes and that small fractions of the halogenated hydrocarbons used in industry may be found in the isolated wax. Such halogenated hydrocarbons are freed at the same temperatures heretofore stated for

evolving hydrocarbon gases and oxygen from wax by our method.

The mechanisms herein shown and described in connection with our method of preparing wax for utilizing its thermal expansion properties are for exemplary purposes only. The molten pre-treated wax may be molded under vacuum into solid units of various forms other than the specific shape illustrated herein FIGS. 10 and 11, with or without embedding the heating elements and pistons therein.

We claim:

1. The method of preparing wax for improving its expansion and contraction properties and capacity to impart motion to mechanism by expansion of the wax when encased in a high pressure casing which is subsequently subjected to temperature exceeding the melting point of the wax for the purpose of expanding the encased wax, which comprises pre-heating the wax before encasement to temperature exceeding the melting point of the wax and exceeding the minimum temperature required to evolve hydrocarbon gases and oxygen from the wax and thereby freeing dissolved hydrocarbon gases and oxygen from the wax, maintaining the degassed molten wax under vacuum and preventing absorption of oxygen, and molding the molten degassed wax under vacuum into solidified units, thereby preventing giving off of gases after encasement when the encased wax is heated and contracts by cooling.

2. The method defined by claim 1, in which the wax is pre-heated to a temperature of at least 140° C.

3. The method defined by claim 1, in which the wax is pre-heated to a temperature of at least 95° C. under high vacuum.

4. The method of preparing paraffin wax for improving its expansion and contraction properties and capacity to impart motion to mechanism by expansion of the wax when encased in a high pressure casing which subsequently is subjected to temperature exceeding the melting point of the wax for the purpose of expanding the encased wax, which comprises selecting a fraction of the wax having melting points in the 54°-60° C. range, pre-heating the wax before encasement to temperature exceeding the melting point of the wax and exceeding the minimum temperature required to evolve hydrocarbon gases and oxygen from the wax and thereby freeing dissolved hydrocarbon gases and oxygen from the wax, maintaining the degassed molten wax under vacuum and preventing absorption of oxygen, and molding the molten degassed wax under vacuum into solidified units, thereby preventing giving off of gases after encasement when the encased wax is heated and contracts by cooling.

5. The method defined by claim 4, in which the wax is pre-heated to a temperature of at least 140° C.

6. The method defined by claim 4, in which the wax is pre-heated to a temperature of at least 95° C. under high vacuum.

7. The method of preparing paraffin wax for improving its expansion and contraction properties and capacity to impart motion to mechanism by expansion of the wax when encased in a high pressure cylinder which subsequently is subjected to temperature exceeding the melting point of the wax for the purpose of expanding the encased wax, which comprises pre-heating the wax before encasement to temperature exceeding the melting point of the wax and exceeding the minimum temperature required to evolve hydrocarbon gases and oxygen from the wax and thereby freeing dissolved hydrocarbon gases and oxygen from the wax, maintaining the degassed molten wax under vacuum and preventing absorption of oxygen, passing the molten degassed wax under vacuum into a mold cavity which contains an electrical heating unit and a piston, filling the entire cavity with the wax and embedding said heating unit and piston, allowing the wax to solidify under vacuum, thereby preventing giving off of gases after encasement when the encased wax is heated and contracts

by cooling, removing the molded wax and parts embedded therein and encasing the molded unit in a high pressure cylinder.

## References Cited by the Examiner

## UNITED STATES PATENTS

1,394,034 10/21 McVickar.  
1,652,212 12/27 Priess ----- 18-59 X  
2,461,723 2/49 Cowan.

2,477,273 7/49 Tognola ----- 18-59  
2,815,035 12/57 Eskin et al. ----- 60-23  
2,815,642 12/57 Sherwood ----- 60-23  
2,846,599 8/58 McAdam ----- 18-59 X

ROBERT F. WHITE, Primary Examiner.

WILLIAM J. STEPHENSON, MICHAEL V. BRINDISI,  
MORRIS LIEBMAN, ALEXANDER H. BROD-  
MERKEL, Examiners.